

## UNITED STATES PATENT OFFICE.

HENRY DREYFUS, OF LONDON, ENGLAND.

## FILAMENTS OR THREADS OF CELLULOSE DERIVATIVES AND METHOD OF MAKING SAME.

No Drawing. Application filed September 16, 1926, Serial No. 136,000, and in Great Britain March 29, 1926.

This invention relates to the manufacture of filaments or threads from cellulose ethers or cellulose esters, particularly cellulose acetates, and to woven, knitted or other fabrics 5 derivable therefrom by any usual textile operation.

In the manufacture of cellulose acetate or other cellulose esters, it is customary, after the acetylation or esterification is complete, to 10 subject the resulting product to a secondary or ripening treatment for the purpose of imparting to it the solubility characteristics requisite for the production of solutions suitable for the manufacture of filaments, for example, by the dry spinning or evaporative 15 method, or by any other appropriate method.

The viscosity of the ripened cellulose acetate—as measured for example by comparison of the rate of flow of a 6% solution 20 in pure acetone at a temperature of 60° F. with the rate of flow of pure glycerine under like conditions, the rate of flow of the glycerine being taken as 100—varies to a marked extent in accordance with the manner in 25 which the cellulose esters are prepared. In order to make an accurate comparison of the relative viscosities of different cellulose esters prepared by different methods the stage at which the ripening is stopped—must be the 30 same for all. The various stages of ripening are shown by the solubility of the cellulose esters in different solvents. In the case of cellulose acetates, the solvents used include acetones, alcohol, benzol-alcohol, and chloroform, 35 alcohol, the most important being benzol-alcohol.

My earlier British Patents Nos. 6,463 of 1915 and 14,101 of 1915 and my U. S. Patents Nos. 1,278,885 and 1,280,975 describe cellulose 40 esters, particularly cellulose acetates, which were the most viscous then known and which can only be produced by the processes described and claimed in these specifications, said cellulose acetates or other esters varying 45 in viscosity from about 20 to 100 or even more, but usually being about 20 to 30 in the case of acetates intended for the production of spinning solutions for use in making filaments of artificial silk.

50 In my British Patent No. 207,562 and my U. S. Patent Application S. No. 633,016 of 18 April, 1923, I described cellulose acetates

which, both before and after ripening in the ordinary way, are of enormously high viscosity, going up to 200, 300 and 400, and even 55 higher.

These products are very valuable as they consist of cellulose acetates in which the original cellulose molecule is much more preserved than in the acetates previously known. While 60 however, these acetates after ripening in the usual manner are soluble in solvents such as acetone to form solutions of the requisite concentration for technical use, ranging, for example, from 10% to 20% or 25% or 30% or 65 even greater concentration, the resulting solutions are of very high viscosity.

I have now found that spinning solutions made from cellulose acetates of very high viscosity can be improved by the addition of 70 small proportions of solvents or plasticisers, such for example as triacetine and diacetine, of higher boiling point than the volatile solvents usually employed in the manufacture of 75 spinning solutions.

According to this invention therefore in making spinning solutions from cellulose ethers or cellulose esters, particularly cellulose acetates, of a viscosity exceeding about 50, and especially cellulose acetates having a 80 viscosity over about 100 for instance 150, 200 or 400, there is incorporated in the spinning solution a small proportion of a solvent or plasticiser of higher boiling point than the volatile solvent or solvents used in the spinning 85 solution.

Particularly of interest are the results which have been obtained by the use of high boiling solvents which have a higher solvent 90 power for cellulose esters than the volatile solvent employed in making the spinning solution, that is to say, high boiling solvents the addition of which to the spinning solution may also lower its viscosity. The higher the solvent power of the added high boiling solvent, 95 the greater is its influence on the spinning qualities of the spinning solution.

Any high boiling solvents or plasticisers for cellulose ethers or esters that are soluble 100 in the spinning solution may be used; for instance, in making spinning solutions containing cellulose acetate of very high viscosity, triacetine, diacetine, mono oil, methyl (or ethyl) toluene (or xylene) sulphonamide, or

other known high boiling solvents or plasticifiers may be employed.

The quantity of high boiling solvent or plasticiser is of importance. It is found that as the quantity of high boiling solvent or plasticiser added is increased from zero upwards, a particular stage is reached beyond which the strength of the filaments decreases gradually thereafter with successive increments in the quantity of high boiling solvent or plasticiser in the spinning solution.

As a general indication it may be stated that in the case of cellulose acetate the proportion of high boiling solvent or plasticiser usually employed does not exceed about 5% though it may sometimes reach 10% or 15% and preferably is about  $\frac{1}{2}$  to 5% by weight of the cellulose acetate.

The proportion of high boiling solvent or plasticiser added to the spinning solution, however, depends upon the grade of cellulose acetate or other cellulose derivative used and upon the nature of the high boiling solvent or plasticiser. Broadly speaking, in the case of solvents or plasticisers which are not evaporated to a substantial extent by dry spinning under ordinary conditions, proportions ranging up to about 5% or occasionally 10%, and preferably of about  $\frac{1}{2}$  to 3% or 5% by weight of the cellulose derivative are employed. In the case of solvents or plasticisers that volatilize to some extent during the spinning operation, larger proportions may be adopted.

In applying these general indications to any particular case, it must be borne in mind that the quantity of high boiling solvent or plasticiser employed depends on the quality of the cellulose acetate or other cellulose derivative and the nature of the high boiling solvent or plasticiser, and particularly on its solvent power for the cellulose derivative. The amount actually employed should be carefully chosen so that the filaments obtained by spinning the resulting solutions do not show a substantial decrease in strength. The spinning solutions so prepared may be extruded through jets into a gaseous atmosphere in which the filaments are solidified by evaporation of the acetone or other volatile solvents employed, or may be spun into filaments in any other appropriate manner.

The resulting filaments may be treated for the complete or partial removal of high boiling solvent or plasticiser by washing or extraction with a liquid which is a non-solvent for the cellulose derivative but which is capable of removing or dissolving the high boiling solvent or plasticifier. When water soluble solvents or plasticifiers such as triacetine, diacetine etc. are used, a simple washing-operation is sufficient for their removal. Methyl (or ethyl) toluene (or xylene) sulphonamide similarly can be removed by

scouring with dilute alkali. The washing out or extraction of the high boiling solvent or plasticiser is preferably effected when the artificial silk is in the form of yarns, but may be performed after the silk has been manufactured into woven or other fabrics.

As high boiling solvents or plasticisers, diacetine, triacetine and the aforementioned sulphonamides have proved to be of considerable value since they are sufficiently soluble in water or dilute alkali to enable them to be removed by an ordinary washing operation.

The high boiling solvents or plasticifiers, especially if present in very small proportions only, may be allowed to remain in the filaments, but an increase in the strength of the filaments is found after the filaments have been washed and dried.

The filaments or threads produced in accordance with this invention, particularly when obtained by dry spinning processes, are of great technical value for the textile industries, being of very great strength, especially after the treatment for the removal of the high-boiling solvent or plasticiser. Indeed, the filaments are much stronger than any artificial filaments previously produced, as might be expected from the very high viscosity of the cellulose derivatives used.

The manner in which the invention can be carried into effect can be illustrated by the following examples, it being understood that these are given only by way of illustration and can be varied widely.

#### Example 1.

100 parts by weight of cellulose are treated with 900 to 1000 parts by weight of glacial acetic acid, 200 to 250 parts by weight of acetic anhydride, and 3 to 10 parts by weight of sulphuric acid at an initial temperature of 0-5° C. which may be allowed to rise to 10 to 15° C. or even higher towards the close of the acetylation. When the acetylation is complete, the excess of acetylating agent is destroyed by the addition of water and the mixture is allowed to stand at about 20° C., until the required solubility characteristics are developed. The acetylation solution can also be treated by neutralizing the effect of the condensing agent partially or completely and afterwards conducting the secondary treatment either at ordinary temperature or with heating to accelerate the reaction as described in my U. S. Patent No. 1,217,722.

100 grams of cellulose acetate prepared in the manner described above are dissolved in about 300 to 500 grams of acetone, and between about 1 to 5 grams of triacetine or mono-oil, or of the aforementioned sulphonamides are added to the resulting solution.

#### Example 2.

100 grams of cellulose acetate prepared as

described in Example 1, are dissolved in about 700 to 900 grams of acetone, and between about 2 to 5 grams of diacetone are added to the solution.

5 The filaments or threads obtained in accordance with this invention, after the removal of the high boiling solvent or plasticiser for example by washing, are of greater strength than any previously obtained, 10 threads having been produced with strengths of 1.4, 1.8, 2, and even 2.2 or more times the strength of any previously known threads made from cellulose acetate.

While as above stated, this invention relates principally to the incorporation of high boiling solvents or plasticisers in spinning solutions containing cellulose derivatives of every high viscosity, it is also possible to produce similar results, though in a smaller degree, by the addition to the spinning solutions of high boiling liquids that are non-solvents for the cellulose derivatives, but are soluble in the spinning solutions, such, for example, as oils.

25 While the invention has been described more particularly with reference to the high viscosity acetates obtained in accordance with my British Patent No. 207,562 and my U. S. Patent Application S. No. 633,016 of 18th 30 April, 1923, it is to be understood that it is applicable generally to cellulose acetates and other cellulose esters and cellulose ethers of very high viscosity as hereinbefore described.

It is also to be understood that the invention includes not only the filaments and threads produced from the new spinning solutions herein described, but also woven, knitted or other fabrics made from or containing such filaments or threads.

35 10 What I claim and desire to secure by Letters Patent is:—

1. A process for the manufacture of artificial filaments or threads from organic substitution derivatives of cellulose of viscosities exceeding about 50, which comprises spinning 45 solutions of said cellulose derivatives comprising less than about 15% calculated on the weight of the cellulose derivatives of a high boiling liquid that is not completely removed 50 during the spinning operation.

2. A process for the manufacture of artificial filaments or threads from cellulose esters of viscosities exceeding about 50, which comprises spinning solutions of said cellulose esters comprising less than about 15% calculated 55 on the weight of the cellulose esters of a high boiling liquid that is not completely removed during the spinning operation.

3. A process for the manufacture of artificial filaments or threads from organic substitution derivatives of cellulose of viscosities exceeding about 50, which comprises dry spinning 60 solutions of said cellulose derivatives in volatile solvents, said solutions comprising less than about 15% calculated on the weight of the 65 cellulose acetates of a high boiling plasticiser for said cellulose acetates, and removing the

of the cellulose derivatives of a high boiling liquid that is not completely volatilized during the spinning operation.

4. A process for the manufacture of artificial filaments or threads from organic substitution derivatives of cellulose of viscosities exceeding about 50, which comprises dry spinning 70 solutions of said cellulose derivatives in volatile solvents, said solutions comprising less than about 15% calculated on the weight 75 of the cellulose derivatives of a high boiling plasticiser for said cellulose derivatives that is not completely volatilized during the spinning operation.

5. A process for the manufacture of artificial filaments or threads from cellulose esters of viscosities exceeding about 50, which comprises dry spinning 80 solutions of said cellulose esters in volatile solvents, said solutions comprising less than about 15% calculated 85 on the weight of the cellulose esters of a high boiling plasticiser for said cellulose esters that is not completely volatilized during the spinning operation.

6. A process for the manufacture of artificial filaments or threads from cellulose acetates of viscosities exceeding about 100, which comprises dry spinning 90 solutions of said cellulose acetates in volatile solvents, said solutions comprising less than about 15% calculated 95 on the weight of the cellulose acetates of a high boiling solvent for said cellulose acetates that is not completely volatilized during the spinning operation.

7. A process for the manufacture of artificial filaments or threads from organic substitution derivatives of cellulose of viscosities exceeding about 50, which comprises spinning 100 solutions of said cellulose derivatives comprising less than about 15% calculated 105 on the weight of the cellulose derivatives of a high boiling liquid, and removing the high boiling liquid from the resulting filaments or threads after the completion of the spinning operation.

8. A process for the manufacture of artificial filaments or threads from cellulose esters of viscosities exceeding about 50, which comprises dry spinning 110 solutions of said cellulose esters in volatile solvents, said solutions comprising less than about 15% calculated on the weight of the cellulose esters of a high boiling plasticiser for said cellulose esters, and removing the plasticiser from the resulting filaments or threads after 115 the completion of the spinning operation.

9. A process for the manufacture of artificial filaments or threads from cellulose acetates of viscosities exceeding about 100, which comprises dry spinning 120 solutions of said cellulose derivative acetates in volatile solvents, said solutions comprising less than about 15% calculated on the weight of the cellulose acetates of a high boiling plasticiser 125 for said cellulose acetates, and removing the 130

plasticiser from the resulting filaments or threads after the completion of the spinning operation.

10. A process for the manufacture of artificial filaments or threads from organic substitution derivatives of cellulose of viscosities exceeding about 50, which comprises dry spinning solutions of said cellulose derivatives in volatile solvents, said solutions comprising a small proportion of a high-boiling plasticiser for said cellulose derivatives, and removing the plasticiser from the resulting filaments or threads by washing.

11. A process for the manufacture of artificial filaments or threads from cellulose acetates of viscosities exceeding about 100, which comprises dry spinning solutions of said cellulose acetates in volatile solvents, said solutions comprising a small proportion of a high-boiling plasticiser for said cellulose acetates, and removing the plasticiser from the resulting filaments or threads by washing.

12. A process for the manufacture of artificial filaments or threads from organic substitution derivatives of cellulose of viscosities exceeding about 50, which comprises dry spinning solutions of said cellulose derivatives in volatile solvents, said solutions comprising from about 1/2% to about 5%, calculated on the weight of the cellulose derivatives, of a high boiling liquid that is not completely volatilized during the spinning operation.

13. A process for the manufacture of artificial filaments or threads from cellulose acetates of viscosities exceeding about 50, which comprises dry spinning solutions of said cellulose acetates in volatile solvents, said solutions comprising from about 1/2% to about 5%, calculated on the weight of the cellulose acetates, of a high boiling solvent for said cellulose acetates that is not completely volatilized during the spinning operation.

14. A process for the manufacture of artificial filaments or threads from cellulose acetates of viscosities exceeding about 50, which comprises dry spinning solutions of said cellulose acetates in volatile solvents, said solutions comprising less than about 10% of a high-boiling liquid, calculated on the weight of the cellulose acetates, and removing the high-boiling liquid from the resulting filaments or threads after the completion of the spinning operation.

15. A process for the manufacture of artificial filaments or threads from cellulose acetates of viscosities exceeding about 50, which comprises dry spinning solutions of said cellulose acetates in volatile solvents, said solutions comprising less than about 10% of a high-boiling solvent for said cellulose acetates, calculated on the weight of the cellulose acetates, and removing the high-boiling

solvent from the resulting filaments or threads by washing.

16. A process for the manufacture of artificial filaments or threads from cellulose acetates of viscosities exceeding about 50, which comprises dry spinning solutions of said cellulose acetates in volatile solvents, said solutions comprising from about 1/2% to about 5% of a high-boiling solvent for said cellulose acetates, calculated on the weight of the cellulose acetates, and removing the high-boiling solvent from the resulting filaments or threads after the completion of the spinning operation.

17. A process for the manufacture of artificial filaments or threads from organic substitution derivatives of cellulose of viscosities exceeding about 50, which comprises producing filaments or threads containing a small proportion of high-boiling liquid, and removing the high-boiling liquid from the filaments or threads after the completion of the spinning operation.

18. A process for the manufacture of artificial filaments or threads from organic substitution derivatives of cellulose of viscosities exceeding about 50, which comprises producing filaments or threads containing a small proportion of high-boiling plasticiser for said cellulose derivatives, and removing the high-boiling plasticiser from the resulting filaments or threads after the completion of the spinning operation.

19. A process for the manufacture of artificial filaments or threads from organic substitution derivatives of cellulose of viscosities exceeding about 50, which comprises producing filaments or threads containing less than about 10% of high-boiling plasticiser for said cellulose derivatives, and removing the high-boiling plasticiser from the filaments or threads after the completion of the spinning operation.

20. A process for the manufacture of artificial filaments or threads from organic substitution derivatives of cellulose of viscosities exceeding about 50, which comprises producing filaments or threads containing between about 1/2% to 3% of high-boiling plasticiser for said cellulose derivatives, and afterwards removing the plasticiser from the filaments by washing.

21. A process for the manufacture of artificial filaments or threads from cellulose acetates of viscosities exceeding about 50, which comprises producing filaments or threads containing less than about 10% of high-boiling plasticiser for said cellulose acetates, and removing the high-boiling plasticiser from the filaments or threads after the completion of the spinning operation.

22. A process for the manufacture of artificial filaments or threads from cellulose acetates of viscosities exceeding about 50, which comprises dry spinning solutions of said cel-

- lulose acetates in volatile solvents, said solutions comprising less than about 10% of a polyacetyl derivative of glycerine, calculated on the weight of the cellulose acetates.
23. A process for the manufacture of artificial filaments or threads from cellulose acetates of viscosities exceeding about 50, which comprises dry spinning solutions of said cellulose acetates in volatile solvents, said solutions comprising between about  $\frac{1}{2}\%$  and about 3% of a polyacetyl derivative of glycerine, calculated on the weight of the cellulose acetates.
24. A process for the manufacture of artificial filaments or threads from cellulose acetates of a viscosity exceeding about 50, which comprises dry spinning solution of said cellulose acetates in volatile solvents, said solutions comprising between about  $\frac{1}{2}\%$  and about 5% of a polyacetyl derivative of glycerine calculated on the weight of the cellulose acetates, and removing the polyacetyl derivative of glycerine from the resulting filaments or threads by washing.
25. Artificial filaments or threads comprising an organic substitution derivative of cellulose of a viscosity exceeding about 50, and less than about 10% of a high-boiling plasticiser for said cellulose derivative.
26. Artificial filaments or threads comprising a cellulose ester of a viscosity exceeding about 50, and between about  $\frac{1}{2}\%$  to 5% of a high-boiling plasticiser for said cellulose ester.
27. Artificial filaments or threads comprising a cellulose acetate of a viscosity exceeding about 100 and between about  $\frac{1}{2}\%$  to about 3% of a polyacetyl derivative of glycerine.
28. A process for the manufacture of artificial filaments or threads from organic substitution derivatives of cellulose of high viscosity which comprises spinning solutions of said cellulose derivatives containing a substance that is a solvent for said cellulose derivatives and which is not volatile at the spinning temperature.
29. A process for the manufacture of artificial filaments or threads from cellulose acetate of high viscosity which comprises spinning solutions of said cellulose acetate containing a substance which is a solvent for said cellulose acetate and which is not volatile at the spinning temperature.
30. A process for the manufacture of artificial filaments or threads from organic substitution derivatives of cellulose of viscosities exceeding about 50 which comprises spinning solutions of said cellulose derivatives containing a substance that is a solvent for said cellulose derivatives and which is not volatile at the spinning temperature.
31. A process for the manufacture of artificial filaments or threads from cellulose acetate of viscosities exceeding about 50, which comprises spinning solutions of said cellulose acetate containing a substance that is a solvent for said cellulose acetate and which is not volatile at this spinning temperature.
- In testimony whereof I have hereunto subscribed my name.
- HENRY DREYFUS.